# EUROPEAN PATENT SPECIFICATION

(11) **EP 3 760 774 B1**
(45) Date of publication and mention of the grant of the patent: **11.09.2024**
(21) Application number: 19909629.8
(22) Date of filing: 20.09.2019
(51) Int. Cl.: D02G 3/02, D02G 3/26, D04H 3/033, D04H 3/007, D01D 5/42, D01D 10/02, D01D 5/00, D01F 6/18, D02G 3/06

(54) **PREPARATION METHOD FOR LONG CONTINUOUS ELECTROSPUN POLYACRYLONITRILE NANOFIBER YARN, AND APPLICATION THEREOF**
VERFAHREN ZUR HERSTELLUNG EINES LANGEN KONTINUIERLICHEN ELEKTROGESPONNENEN POLYACRYLNITRILNANOFASERGARNS UND DESSEN ANWENDUNG
PROCÉDÉ DE PRÉPARATION DE FIL DE NANOFIBRES DE POLYACRYLONITRILE ÉLECTROFILÉES LONGUES CONTINUES ET APPLICATION ASSOCIÉE

(30) Priority: 21.05.2019 CN 201910422360
(43) Date of publication of application: 06.01.2021
(73) Proprietor: JIANGXI ADVANCED NANOFIBER S&T CO., LTD, High-Tech District Nanchang Jiangxi 330096 (CN)
(72) Inventor: HOU, Haoqing, Nanchang Jiangxi 330096 (CN); OUYANG, Wen, Nanchang Jiangxi 330096 (CN); WANG, Yuming, Nanchang Jiangxi 330096 (CN); CHENG, Chuyun, Nanchang Jiangxi 330096 (CN); WANG, Qi, Nanchang Jiangxi 330096 (CN); LV, Xiaoyi, Nanchang Jiangxi 330096 (CN)
(74) Representative: Schlich, George
(86) International application number: PCT/CN2019/106959
(87) International publication number: WO 2020/232931

(56) References cited:
- EP-A1- 3 187 629
- WO-A1-2005/073442
- CN-A- 103 132 194
- CN-A- 104 947 211
- CN-A- 104 947 211
- CN-A- 105 603 561
- CN-A- 106 120 157
- CN-A- 107 503 000
- CN-A- 107 841 808
- CN-A- 107 858 780
- CN-A- 110 079 903
- CN-A- 110 129 934
- CN-A- 110 144 649
- CN-A- 110 184 684
- US-A1- 2016 298 265

## Description

### Technical Field

The present invention relates to the field of continuous filament yarn of polymer fibers, in particular to a method for preparing a continuous filament yarn of electrospun polyacrylonitrile nanofibers and uses thereof.

### Background

Polyacrylonitrile fiber, commonly known as acrylic fiber or artificial wool, is a commonly used artificial fiber that can be used to replace or blended with wool to make wool fabrics. It has a good effect of warmth retention, and it also has excellent weather resistance and light resistance, after one year of open-air exposure, the intensity only decreases by 20%, so it is often used to make curtains, tarpaulins, etc.

Electrospinning is a special fiber manufacturing process, and has been used more and more in the past ten years to prepare nanofiber materials. Its working method is as follows: the polymer solution or the melt is jetted out in a high-voltage electric field, solidified in a running distance, and finally the spinning is received by a receiving device. Due to the process of electrostatic spinning is simple, and various forms of fibers can also be produced according to demand, such as solid fibers, hollow fibers, core-shell structure fibers, etc., it has broad prospects in many fields. CN104947211A discloses a film-slitting electrostatic spinning continuous nanofiber yarn device and a method for preparing continuous nanofiber yarns by this device.

However, the current electrostatic spinning technology is only used to manufacture a non-woven fabric or spray a thin layer of nano-cobweb on industrial non-woven fabrics (generally with an areal density of about 1 g/m²), which can also manufacture discontinuous and higher linear density of thick yarn, and there is no technology in the world that can continuously manufacture ultra-small linear density or ultra-high count yarn of electrospun nanofibers. The linear density of conventional fiber yarns is above 6 Tex, and the counts of the yarns are generally less than 150 counts, and most of them are below 100 counts.

### Summary

To solve the above technical problems, the first aspect of the present invention provides a method for preparing a continuous filament yarn of electrospun polyacrylonitrile nanofibers, wherein the continuous filament yarn has a length of no less than 2000 meters and a metric count of more than 500, the method comprising the following steps:
a. dissolving a polyacrylonitrile raw material in a polar solvent under mechanical stirring to obtain a uniform spinning solution, wherein a mass concentration of the spinning solution is 12 to 22% (w/w);
b. making the polyacrylonitrile solution in the step a into a polyacrylonitrile nonwoven fabric in an electrospinning machine, wherein the polyacrylonitrile solution is spraying spun in a high-voltage electric field, and DC voltage of the high-voltage electric field in the step b is 30 to 50 kV;
c. cutting the nonwoven fabric in the step b into slender strips with a width of 0.5 to 6 cm;
d. drafting the slender strips in the step c in a water bath at 80 to 95°C with a draft ratio of 2 to 5 times, then drafting in air at 110 to 150°C with a draft ratio of 3 to 10 times to obtain a fiber bundle with highly oriented internal fibers;
e. twisting the fiber bundle in the step d to obtain a continuous filament yarn of electrospun polyacrylonitrile nanofibers with a length of not less than 2000 meters, and the unwinding speed of the twisting is 5 to 50 m/min.

According to a preferred embodiment, the polar solvent in the step a is one or more selected from the group consisting of N, N-dimethylformamide, N-methylpyrrolidone, dimethyl sulfoxide, and N, N-dimethylacetamide.

According to another preferred embodiment, the water bath draft and air draft in the step d are 5-roll drafts.

According to another yet preferred embodiment, the unwinding speed of the water bath draft in the step d is 2 to 8 m/min.

According to another yet preferred embodiment, the unwinding speed of the air draft in the step d is 3 to 8 m/min.

According to another yet preferred embodiment, the fiber orientation degree of the fiber bundle in the step d is 90% to 95%.

According to another yet preferred embodiment, the unwinding speed of twisting in the step e is 5 to 50 m/min.

According to another yet preferred embodiment, the twist degree of twisting in the step e is 500 to 1500 twist/m.

The second aspect of the present invention provides a continuous filament yarn of electrospun polyacrylonitrile nanofibers, which is prepared by the above method for preparing a continuous filament yarn of electrospun polyacrylonitrile nanofibers.

The continuous filament yarn of electrospun polyacrylonitrile nanofibers may be used for pure or blended spinning to weave a light-weight and warm high-grade fabric.

Beneficial effects: the present invention provides a method for preparing a continuous filament yarn of electrospun polyacrylonitrile nanofibers, which enhance the mechanical properties of polyacrylonitrile fibers through draft operation and can produce continuously, and the produced filament yarns have a length of not less than 2000 meters and a metric count of more than 500, which can be used for pure or blended spinning to obtain a light-weight, warm and durable high-grade fabric.

### Detailed Description of The Embodiments

The content of the present invention can be further understood in conjunction with the following detailed description of the preferred implementation methods of the present invention and the included embodiments. Unless otherwise stated, all the technical and scientific terms used herein have the same meaning as commonly understood by those of ordinary skill in the art to which the application belongs. If the definition of a specific term disclosed in the prior art is inconsistent with any definition provided in this application, the definition of the term provided in this application shall prevail.

As used herein, unless the context clearly indicates otherwise, features that do not define singular and plural forms are also intended to include features of the plural form. It should also be understood that, as used herein, the term "prepared from" is synonymous with "comprise", "include", "including", "having", " comprise" and/or "comprising", when used in this specification, they mean the stated composition, step, method, article or device, but do not exclude the presence or addition of one or more other compositions, steps, methods, articles or devices. In addition, when describing the embodiments of the present application, the use of "preferred", "preferably", "more preferably", etc. refers to an embodiment of the present invention that can provide certain beneficial effects under certain circumstances. However, other embodiments may also be preferred under the same or other circumstances. In addition, the expression of one or more preferred embodiments does not imply that other embodiments are not available, nor is it intended to exclude other embodiments from the scope of the present invention.

In order to solve the above technical problems, the present invention provides a method wherein for preparing a continuous filament yarn of electrospun polyacrylonitrile nanofibers, the continuous filament yarn has a length of no less than 2000 meters and a metric count of more than 500, comprising the following steps:
a. dissolving a polyacrylonitrile raw material in a polar solvent under mechanical stirring to obtain a uniform spinning solution, wherein a mass concentration of the spinning solution is 12 to 22% (w/w);
b. making the polyacrylonitrile solution in the step a into a polyacrylonitrile nonwoven fabric in an electrospinning machine, wherein the polyacrylonitrile solution is spraying spun in a high-voltage electric field, and DC voltage of the high-voltage electric field in the step b is 30 to 50 kV; machine;
c. cutting the nonwoven fabric in the step b into slender strips with a width of 0.5 to 6 cm;
d. drafting the slender strips in the step c in a water bath at 80 to 95°C with a draft ratio of 2 to 5 times, then drafting in air at 110 to 150°C with a draft ratio of 3 to 10 times to obtain a fiber bundle with highly oriented internal fibers;
e. twisting the fiber bundle in the step d to obtain a continuous filament yarn of electrospun polyacrylonitrile nanofibers with a length of not less than 2000 meters, and the unwinding speed of the twisting is 5 to 50 m/min.

### Step a

The objective of step a is to prepare a polymer solution suitable for electrostatic spinning, and because there are a large number of polar cyano groups in polyacrylonitrile, selecting a suitable polar solvent helps to prepare a spinning solution with suitable concentration and adjustable viscosity.

Step a. dissolving a polyacrylonitrile raw material in a polar solvent under mechanical stirring to obtain a uniform spinning solution.

In some preferred embodiments, the polyacrylonitrile raw material and the polar solvent are added together in a stainless steel reactor and dissolved under mechanical stirring to obtain a uniform polyacrylonitrile solution for spinning.

The polyacrylonitrile raw material in the present invention is not particularly limited, and may be commercially available, and the CAS number is 25014-41-9.

In some embodiments, the polar solvent in step a is selected from one or more of N, N-dimethylformamide (CAS number: 68-12-2), N-methylpyrrolidone (CAS number: 872-50-4), dimethyl sulfoxide (CAS No. 67-68-5) and N, N-dimethylacetamide (CAS No. 127-19-5).

Both dimethyl sulfoxide and N-methylpyrrolidone are good solvents for dissolving polyacrylonitrile, and dimethyl sulfoxide is non-toxic, but both have boiling points above 200°C, and the spun yarns are not easy to dry and have serious adhesion to each other. N, N-dimethylformamide has the lowest boiling point among several listed solvents and has the best solubility, while N, N-dimethylacetamide has relatively low solubility, but has the advantage of low toxicity which can be compounded with N, N-dimethylformamide to make a mixed solvent for spinning.

In some preferred embodiments, the polar solvent in the step a is N, N-dimethylformamide and/or N, N-dimethylacetamide; further preferably, the N, N-Dimethylformamide and N, N-dimethylacetamide; further, the mass ratio of N, N-dimethylformamide and N, N-dimethylacetamide is 4: 1.

The concentration of the spinning solution determines the viscosity of the solution, if the viscosity is too large, the electrostatic force needs to overcome a greater surface tension, making the spinning diameter too large or even impossible to spin; and too small viscosity will make the spinning too thin, insufficient strength, or beads may appear on the spinning. The mass concentration of the solution in the step a is 12 to 22%; preferably, the mass concentration of the solution in the step a is 13 to 18%,

In some preferred embodiments, the absolute viscosity of the solution in the step a is 1.5 to 5 Pa.S; further preferably, the absolute viscosity of the solution in the step a is 2 to 4 Pa.S.

On the one hand, appropriate dissolution temperature can speed up the dissolution rate and improve the processing efficiency, on the other hand can reduce the solubility of the gas in the solution, and remove the gas from the solution. In some preferred embodiments, the dissolution temperature in the step a is 30 to 55°C, and the stirring time is 4 to 10 hours; further preferably, the dissolution temperature in the step a is 38 to 48°C, and the stirring time is 6 to 9 hours.

### Step b

The objective of the step b is to make polyacrylonitrile from solution into a nonwoven fabric, in this process, the polymer solution is sprayed into a strong electric field. Under the action of the electric field, the sprayed droplets change from spherical to Taylor cone, from the tip of which a tiny jet is extended, and after running for a certain distance, the jet is solidified into fiber filaments, which are collected by a stainless steel mesh belt to obtain a nonwoven fabric.

Step b. making the polyacrylonitrile solution in the step a into a polyacrylonitrile nonwoven fabric in an electrospinning machine.

The polyacrylonitrile solution is injected into the spinning device of an electrospinning machine, spraying spun in a high-voltage electric field, and collected with a stainless steel mesh belt to obtain an electrospun polyacrylonitrile nonwoven fabric.

The magnitude of the voltage of the electric field will affect the shape of the sprayed droplets. Too small voltage cannot make the spherical droplets of the spinneret form a Taylor cone, and too large voltage will cause the formed Taylor cone to retreat or even back into the spinneret, resulting a large number of beads appeared in the spinning fibers. The DC voltage of the high-voltage electric field in the step b is 30 to 50 kV; preferably, the DC voltage of the high-voltage electric field in the step b is 40 to 45 kV,

The distance between the spinneret and the stainless steel mesh belt collector requires to ensure that the jet can be solidified during running without adhesion, and improper receiving distance will cause beads appeared in the spinning fibers. In some preferred embodiments, the distance between the spinneret and the stainless steel mesh belt collector in the step b is 25 to 55 cm; further preferably, the distance between the spinneret and the stainless steel mesh belt collector is 28 to 35 cm.

The travel speed of the stainless steel mesh belt can affect the pore size and thickness of the nonwoven fabric, which in turn affects the strength of the filament yarn processed from the nonwoven fabric. In some preferred embodiments, the travel speed of the stainless steel mesh belt in the step b is 1 to 5 m/min; further preferably, the travel speed of the stainless steel mesh belt is 2 to 4 m/min.

In some preferred embodiments, the diameter of the spinning in step b is 100-1500 nm; further preferably, the diameter of the spinning in the step b is 100 to 500 nm.

### Step c

The objective of the step c is to pretreat the polyacrylonitrile nonwoven fabric into a form suitable for further processing.

Step c: cutting the nonwoven fabric in the step b into slender strips with a width of 0.5 to 6 cm.

The width of the cut strip will affect the subsequent further processing, and too narrow cut strip is not conducive to continuous production, making the resulting yarn easily broken, and it is impossible to achieve the ideal length to obtain a filament yarn; while too wide cut strip is difficult to process to obtain a fiber bundle with highly oriented internal fibers. The width of the slender strip in the step c is 0.5 to 6 cm; preferably, the width of the slender strip is 2 to 5.5 cm.

### Step d

The objective of the step d is, on the one hand, to obtain a fiber bundle length sufficient to produce continuous filament yarns through drafting, and on the other hand, to change the degree of orientation of the internal fibers, making the strength of the fiber bundle in the orientation direction increased greatly-.

Step d: drafting the slender strips in the step c in a water bath at 80 to 95°C with a draft ratio of 2 to 5 times, then drafting in air at 110 to 150°C with a draft ratio of 3 to 10 times to obtain a fiber bundle with highly oriented internal fibers.

In some preferred embodiments, the water bath draft and air draft in the step d are 5-roll drafts.

In some preferred embodiments, the unwinding speed of the water bath draft is 2 to 8 m/min; further preferably, the unwinding speed of the water bath draft is 4 to 7 m/min.

In some preferred embodiments, the unwinding speed of the air draft is 3 to 8 m/min; further preferably, the unwinding speed of the air draft is 4 to 7 m/min.

In some preferred embodiments, the fiber orientation degree of the fiber bundle in the step d is 90% to 95%.

### Step e

The objective of the step e is to twist the fiber bundle into a filament yarn. After twisting, the outer fiber and the inner fiber squeeze each other to generate pressure, making the yarn obtain frictional force along the fiber length, and the fiber strip is longitudinally fixed, and the fiber after yarn formation has improved properties such as strength, elongation, gloss, and feel.

Step e: twisting the fiber bundle in the step d to obtain a continuous filament yarn of electrospun polyacrylonitrile nanofibers with a length of not less than 2000 meters.

The unwinding speed of twisting in the step e is 5 to 50 m/min; preferably, the unwinding speed of twisting is 20 to 40 m/min,

In some preferred embodiments, the twist degree of twisting in the step e is 500 to 1500 twist/m; further preferably, the twist degree of twisting in the step e is 800 to 1200 twist/m.

Compared with other fibers, the strength of polyacrylonitrile nanofibers is lower. In terms of the original excellent properties of polyacrylonitrile such as weather resistance and warmth retention, the strength of polyacrylonitrile fiber after high drafting is further improved, which broadens its range of application. After the fiber is drafted and twisted, filament yarn can be produced continuously, which in turn can be used for pure or blended with other fibers to weave alight-weight, warm, soft, and comfortable high-grade fabric.

### Examples

The technical solutions of the present invention will be described in detail below through the examples, but the protection scope of the present invention is not limited to the examples.

### Example 1

Example 1 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric. The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 88°C with an unwinding speed of twisting of 6 m/min and a draft ratio of 3 times, then 5-roll drafting in air at 135°C with an unwinding speed of twisting of 6 m/min and a draft ratio of 6 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 2

Example 2 provided a method for preparing a continuous filament yarn of electrospun polyacrylonitrile nanofibers, comprising the following steps:
dissolving a polyacrylonitrile raw material and N, N-dimethylformamide in a stainless steel reaction reactor under mechanically stirring, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric. The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 88°C with an unwinding speed of twisting of 6 m/min and a draft ratio of 3 times, then 5-roll drafting in air at 135°C with an unwinding speed of twisting of 6 m/min and a draft ratio of 6 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 3

Example 3 provided a method for preparing a continuous filament yarn of electrospun polyacrylonitrile nanofibers, comprising the following steps:
dissolving a polyacrylonitrile raw material and N, N-dimethylacetamide in a stainless steel reaction reactor under mechanically stirring, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 88°C with an unwinding speed of twisting of 6 m/min and a draft ratio of 3 times, then 5-roll drafting in air at 135°C with an unwinding speed of twisting of 6 m/min and a draft ratio of 6 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 4

Example 4 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 2 cm;
5-roll drafting the slender strips in the step c in a water bath at 88°C with an unwinding speed of twisting of 6 m/min and a draft ratio of 3 times, then 5-roll drafting in air at 135°C with an unwinding speed of twisting of 6 m/min and a draft ratio of 6 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 5

Example 5 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 5.5 cm;
5-roll drafting the slender strips in the step c in a water bath at 88°C with an unwinding speed of twisting of 6 m/min and a draft ratio of 3 times, then 5-roll drafting in air at 135°C with an unwinding speed of twisting of 6 m/min and a draft ratio of 6 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 6

Example 6 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 88°C with an unwinding speed of twisting of 6 m/min and a draft ratio of 5 times to obtain a fiber bundle of electrospun polyacrylonitrile;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 7

Example 7 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 88°C with an unwinding speed of twisting of 6 m/min and a draft ratio of 2 times, then 5-roll drafting in air at 135°C with an unwinding speed of twisting of 6 m/min and a draft ratio of 3 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 8

Example 8 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 88°C with an unwinding speed of twisting of 6 m/min and a draft ratio of 5 times, then 5-roll drafting in air at 135°C with an unwinding speed of twisting of 6 m/min and a draft ratio of 10 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 9

Example 9 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 80°C with an unwinding speed of twisting of 6 m/min and a draft ratio of 3 times, then 5-roll drafting in air at 110°C with an unwinding speed of twisting of 6 m/min and a draft ratio of 6 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Example 10

Example 10 provided a method for preparing a continuous filament yarn of electrospun polyacrylonitrile nanofibers, comprising the following steps:
dissolving a polyacrylonitrile raw material and a mixed solvent composed of N, N-dimethylformamide and N, N-dimethylacetamide in a stainless steel reaction reactor under mechanically stirring, and the mass ratio of N, N-dimethylformamide and N, N-dimethylacetamide was 4: 1, the dissolution temperature was 43°C., the stirring time was 8 hours. and the mass concentration of the obtained polyacrylonitrile solution for spinning was 15%;
injecting the solution obtained in the step a into the spinning device of an electrostatic spinning machine, spraying spun in a high-voltage electric field with a DC voltage of 42 kV, and collected with a stainless steel mesh belt to obtain an electrospun polyacrylonitrile nonwoven fabric, The distance between the spinneret and the stainless steel mesh belt collector was 33 cm, the travel speed of the stainless steel mesh belt was 3 m/min, and the diameter of the spinning was 150 nm;
cutting the nonwoven fabric in the step b into slender strips with a width of 4 cm;
5-roll drafting the slender strips in the step c in a water bath at 95°C with an unwinding speed of twisting of 6 m/min and a draft ratio of 3 times, then 5-roll drafting in air at 150°C with an unwinding speed of twisting of 6 m/min and a draft ratio of 6 times to obtain a fiber bundle of electrospun polyacrylonitrile with highly oriented internal fibers;
twisting the fiber bundle in the step d to more than 2000 meters, the unwinding speed was 25 m/min, and the twist degree was 900 twist/m to obtain a continuous filament yarn of electrospun polyacrylonitrile nanofibers.

### Performance evaluation

The continuous filament yarns of electrospun polyacrylonitrile nanofibers obtained in examples 1 to 10 were tested for metric count, tensile strength, Young's modulus, and elongation at break.

Metric count,: 1000 meters of yarn was weighed its gram weight, and the metric count = 1000/gram weight. The results were shown in Table 1.

Tensile strength, Young's modulus, elongation at break: tested with an electronic universal tensile machine. The results were shown in Table 1.

**Table 1**

| | Metric count | Tensile strength | Young's modulus | Elongation at break |
|---|---|---|---|---|
| Example 1 | 740 | 15 cN/dtex | 298 cN/dtex | 11% |
| Example 2 | 720 | 14.5 cN/dtex | 290 cN/dtex | 12% |
| Example 3 | 660 | 12 cN/dtex | 246 cN/dtex | 19% |
| Example 4 | 760 | 3 cN/dtex | 84 cN/dtex | 12% |
| Example 5 | 700 | 13 cN/dtex | 260 cN/dtex | 14% |
| Example 6 | 450 | 6 cN/dtex | 108 cN/dtex | 32% |
| Example 7 | 520 | 11.5 cN/dtex | 223 cN/dtex | 27% |
| Example 8 | 800 | 8 cN/dtex | 130 cN/dtex | 10% |
| Example 9 | 630 | 10 cN/dtex | 194 cN/dtex | 22% |
| Example 10 | 600 | 9.5 cN/dtex | 172 cN/dtex | 17% |

It can be known from the comparison of examples 1 to 10 that the method for preparing a continuous filament yarn of electrospun polyacrylonitrile nanofibers can produce a high count filament yarn with a length of more than 2000 meters, while improving the mechanical properties of the polyacrylonitrile fiber. Finally, it is pointed out that the foregoing is only preferred exemplary embodiments of the which is present invention and is not intended to be limiting of the present invention, defined by the claims.

## Claims

1. A method for preparing a continuous filament yarn of electrospun polyacrylonitrile nanofibers, wherein the continuous filament yarn has a length of no less than 2000 meters and a metric count of more than 500, the method comprising the following steps:
a. dissolving a polyacrylonitrile raw material in a polar solvent under mechanical stirring to obtain a uniform spinning solution, wherein a mass concentration of the spinning solution is 12 to 22% (w/w);
b. making the polyacrylonitrile solution in the step a into a polyacrylonitrile nonwoven fabric in an electrospinning machine, wherein the polyacrylonitrile solution is spraying spun in a high-voltage electric field, and DC voltage of the high-voltage electric field in the step b is 30 to 50 kV;
c. cutting the nonwoven fabric in the step b into slender strips with a width of 0.5 to 6 cm;
d. drafting the slender strips in the step c in a water bath at 80 to 95°C with a draft ratio of 2 to 5 times, then drafting in air at 110 to 150°C with a draft ratio of 3 to 10 times to obtain a fiber bundle with highly oriented internal fibers;
e. twisting the fiber bundle in the step d to obtain a continuous filament yarn of electrospun polyacrylonitrile nanofibers with a length of not less than 2000 meters, and the unwinding speed of the twisting is 5 to 50 m/min.

2. The method for preparing the continuous filament yarn of electrospun polyacrylonitrile nanofibers according to claim 1, wherein the polar solvent in the step a is selected from one or more of N, N-dimethylformamide, N-methylpyrrolidone, dimethyl sulfoxide, N, N-dimethylacetamide.

3. The method for preparing the continuous filament yarn of electrospun polyacrylonitrile nanofibers according to claim 1 or 2, wherein the water bath draft and the air draft in the step d are 5-roll drafts.

4. The method for preparing the continuous filament yarn of electrospun polyacrylonitrile nanofibers according to any one of claims 1 to 3, wherein the unwinding speed of the water bath draft in the step d is 2 to 8 m/min.

5. The method for preparing the continuous filament yarn of electrospun polyacrylonitrile nanofibers according to any one of claims 1 to 4, wherein an unwinding speed of the air draft in the step d is 3 to 8 m/min.

6. The method for preparing the continuous filament yarn of electrospun polyacrylonitrile nanofibers according to any one of claims 1 to 5, wherein the unwinding speed of twisting in the step e is 5 to 50 m/min.

7. The method for preparing the continuous filament yarn of electrospun polyacrylonitrile nanofibers according to any one of claims 1 to 6, wherein the twist degree of twisting in the step e is 500 to 1500 twist/m.

8. A continuous filament yarn of electrospun polyacrylonitrile nanofibers, which is prepared by the method for preparing the continuous filament yarn of electrospun polyacrylonitrile nanofibers according to any one of claims 1 to 7.

## Patentansprüche

1. Verfahren zur Herstellung eines Endlosfilamentgarns aus elektrogesponnenen Polyacrylnitril-Nanofasern, wobei das Endlosfilamentgarn eine Länge von nicht weniger als 2000 Metern und eine metrische Anzahl von mehr als 500 aufweist, wobei das Verfahren die folgenden Schritte umfasst:
a. Auflösen eines Polyacrylnitril-Rohmaterials in einem polaren Lösungsmittel unter mechanischem Rühren, um eine gleichmäßige Spinnlösung zu erhalten, wobei die Massenkonzentration der Spinnlösung 12 bis 22 % (w/w) beträgt;
b. Umwandeln der Polyacrylnitrillösung aus Schritt a in einen Polyacrylnitrilvliesstoff in einer Elektrospinnmaschine, wobei die Polyacrylnitrillösung in einem elektrischen Hochspannungsfeld sprühgesponnen wird und die Gleichspannung des elektrischen Hochspannungsfelds in Schritt b 30 Volt bis 50 kV beträgt;
c. Schneiden des Vliesstoffs aus Schritt b in schmale Streifen mit einer Breite von 0,5 bis 6 cm;
d. Verstrecken der schlanken Streifen aus Schritt c in einem Wasserbad bei 80 bis 95 °C mit einem Verstreckungsverhältnis von 2 bis 5 mal, dann Verstrecken an Luft bei 110 bis 150 °C mit einem Verstreckungsverhältnis von 3 bis 10 mal, um ein Faserbündel mit hochorientierten Innenfasern zu erhalten; und
e. Verdrillen des Faserbündels aus Schritt d, um ein Endlosfilamentgarn aus elektrogesponnenen Polyacrylnitril-Nanofasern mit einer Länge von nicht weniger als 2000 Metern zu erhalten, wobei die Abspulgeschwindigkeit beim Verdrillen 5 bis 50 m/min beträgt.

2. Verfahren zur Herstellung des Endlosfilamentgarns aus elektrogesponnenen Polyacrylnitril-Nanofasern nach Anspruch 1, wobei das polare Lösungsmittel in Schritt a ausgewählt ist aus einem oder mehreren von N, N-Dimethylformamid, N-Methylpyrrolidon, Dimethylsulfoxid, N, N-Dimethylacetamid.

3. Verfahren zur Herstellung des Endlosfilamentgarns aus elektrogesponnenen Polyacrylnitril-Nanofasern nach Anspruch 1 oder 2, wobei der Wasserbad-Verstreckung und der Luft-Verstreckung im Schritt d 5-Walzen-Verstreckung sind.

4. Verfahren zur Herstellung des Endlosfilamentgarns aus elektrogesponnenen Polyacrylnitril-Nanofasern nach einem der Ansprüche 1 bis 3, wobei die Abspulgeschwindigkeit der Wasserbad-Verstreckung im Schritt d 2 bis 8 m/min beträgt.

5. Verfahren zur Herstellung des Endlosfilamentgarns aus elektrogesponnenen Polyacrylnitril-Nanofasern nach einem der Ansprüche 1 bis 4, wobei die Abspulgeschwindigkeit der Luft-Verstreckung im Schritt d 3 bis 8 m/min beträgt.

6. Verfahren zur Herstellung des Endlosfilamentgarns aus elektrogesponnenen Polyacrylnitril-Nanofasern nach einem der Ansprüche 1 bis 5, wobei die Abspulgeschwindigkeit des Verdrillens im Schritt e 5 bis 50 m/min beträgt.

7. Verfahren zur Herstellung des Endlosfilamentgarns aus elektrogesponnenen Polyacrylnitril-Nanofasern nach einem der Ansprüche 1 bis 6, wobei der Verdrehungsgrad des Verdrillens im Schritt e 500 bis 1500 Verdrehungen/m beträgt.

8. Endlosfilamentgarn aus elektrogesponnenen Polyacrylnitril-Nanofasern, das nach dem Verfahren zur Herstellung des Endlosfilamentgarns aus elektrogesponnenen Polyacrylnitril-Nanofasern nach einem der Ansprüche 1 bis 7 hergestellt ist.

## Revendications

1. Procédé de préparation d'un fil continu de nanofibres de polyacrylonitrile électrofilées, dans lequel le fil continu a une longueur d'au moins 2000 mètres et un nombre métrique supérieur à 500, le procédé comprenant les étapes suivantes:
a. dissolution d'une matière première de polyacrylonitrile dans un solvant polaire sous agitation mécanique pour obtenir une solution de filage uniforme, dans laquelle la concentration massique de la solution de filage est de 12 à 22 % (w/w);
b. transformer la solution de polyacrylonitrile de l'étape a en un tissu non tissé de polyacrylonitrile dans une machine d'électrofilage, la solution de polyacrylonitrile étant filée par pulvérisation dans un champ électrique à haute tension, et la tension continue du champ électrique à haute tension à l'étape b étant comprise entre 30 et 50 kV;
c. couper le tissu non tissé à l'étape b en bandes minces d'une largeur de 0,5 à 6 cm;
d. étirer les bandes minces à l'étape c dans un bain d'eau à 80 à 95°°C avec un rapport de tirage de 2 à 5 fois, puis étirer dans l'air à 110 à 150°°C avec un rapport de tirage de 3 à 10 fois pour obtenir un faisceau de fibres avec des fibres internes fortement orientées;
e. tordre le faisceau de fibres à l'étape d pour obtenir un fil de filament continu de nanofibres de polyacrylonitrile électrofilées d'une longueur d'au moins 2000 mètres, et la vitesse de déroulement de la torsion est de 5 à 50 m/min.

2. Procédé de préparation du fil continu de nanofibres de polyacrylonitrile électrofilées selon la revendication 1, dans lequel le solvant polaire de l'étape a est choisi parmi un ou plusieurs des solvants suivants: N, N-diméthylformamide, N-méthylpyrrolidone, sulfoxyde de diméthyle, N, N-diméthylacétamide.

3. Procédé de préparation du fil continu de nanofibres de polyacrylonitrile électrofilées selon la revendication 1 ou 2, dans lequel le tirage du bain d'eau et le tirage de l'air à l'étape d sont des tirages à 5 rouleaux.

4. Procédé de préparation du fil continu de nanofibres de polyacrylonitrile électrofilées selon l'une quelconque des revendications 1 à 3, dans lequel la vitesse de déroulement de l'étirage du bain d'eau à l'étape d est de 2 à 8 m/min.

5. Procédé de préparation du fil continu de nanofibres de polyacrylonitrile électrofilées selon l'une quelconque des revendications 1 à 4, dans lequel la vitesse de déroulement de l'appel d'air à l'étape d est de 3 à 8 m/min.

6. Procédé de préparation du fil continu de nanofibres de polyacrylonitrile électrofilées selon l'une quelconque des revendications 1 à 5, dans lequel la vitesse de déroulement de la torsion à l'étape e est de 5 à 50 m/min.

7. Procédé de préparation du fil continu de nanofibres de polyacrylonitrile électrofilées selon l'une quelconque des revendications 1 à 6, dans lequel le degré de torsion à l'étape e est compris entre 500 et 1500 torsions/m.

8. Filament continu de nanofibres de polyacrylonitrile électrofilées, préparé par le procédé de préparation du filament continu de nanofibres de polyacrylonitrile électrofilées selon l'une quelconque des revendications 1 à 7.
